

## UNITED STATES PATENT OFFICE

2,096,154

MODIFIED TEXTILE MATERIALS AND  
METHOD OF TREATING SAMEWilliam Whitehead, Cumberland, Md., assignor  
to Celanese Corporation of America, a corpora-  
tion of DelawareNo Drawing. Application May 1, 1935,  
Serial No. 19,200

## 7 Claims. (Cl. 8—5)

This invention relates to the modification of 5  
yarns and other textile materials containing an  
organic derivative of cellulose while the same are  
in transit from a source of supply to a packag-  
ing device or during other winding operations.  
This invention especially relates to the treatment  
in localized areas of yarns containing an ester  
of cellulose with a saponifying agent or other  
modifying agent that contains a substance per-  
mitting the operator to visually ascertain the  
amount and extent of treatment.

An object of the invention is the economic and  
expeditious production of yarns treated with a  
modifying agent, having a color imparting ma-  
terial therein, making visible the amount and  
extent of treatment. Other objects of the invention  
will appear from the following detailed de-  
scription.

By the prior methods of treating yarns or a  
plurality of yarns such as a warp or fabric with  
a modifying agent that has little or no color  
effect on the yarns, one was not able to observe  
the manner in which the treatment was being  
applied. In such processes as the application of  
a saponifying agent to yarns containing an ester  
of cellulose for sensitizing same for future treat-  
ments to develop the saponification, irregulari-  
ties in the application of the saponifying agent  
were often not recognized until the yarns were  
30 formed into a fabric. By applying a saponify-  
ing or other colorless modifying agent in ac-  
cordance with my invention, however, the appli-  
cation of the same may be watched as the same  
is being applied and corrections of irregulari-  
ties in the treatment immediately made.

In accordance with my invention, I treat yarns,  
warps or fabrics with substances that tend to  
modify various properties of the yarn and in-  
corporate with those substances a coloring ma-  
terial that has no affinity for the textile material,  
either before or after the modifying action, for  
the purpose of rendering visible the extent and  
amount of treatment applied to the yarn. Fur-  
ther, in accordance with my invention, I apply to  
textile materials such as yarns, warps and fab-  
rics containing filaments of organic esters of cel-  
lulose a saponifying or sensitizing agent that  
renders the textile materials susceptible to the  
development of saponification by subsequent  
treatments. The sensitizing agent is adapted to  
50 partially saponify the yarns, said agent preferably  
containing a colored organic material having no  
affinity for the textile materials either before  
or after they have been saponified.

55 This invention is applicable to the treatment

of yarn, bands of yarn, fabric or any type of  
textile material where the treating agent ap-  
plied is of the same or similar color to the yarn  
being treated, making it difficult to see the  
amount or extent of treatment. This invention 5  
is applicable to the total, partial, intermittent  
or other types of saponifying actions. This inven-  
tion, however, is of particular importance in the  
saponifying or sensitizing for subsequent devel-  
opment of saponification of yarns containing or-  
ganic esters of cellulose. The invention will be  
described in detail with respect to the saponify-  
ing and sensitizing of yarns, etc. containing or-  
ganic esters of cellulose.

Any suitable organic ester of cellulose may be 15  
employed in the yarn, fabric or warp to be sensi-  
tized or saponified. For example, I may employ  
such organic esters of cellulose as cellulose ace-  
tate, cellulose formate, cellulose butyrate and  
cellulose propionate. Although this invention is 20  
of particular importance in the treatment of  
yarns consisting only of filaments of organic  
esters of cellulose, it nevertheless is applicable  
to yarns formed from a mixture of differing fila-  
ments, such as a mixture of filaments containing 25  
organic esters of cellulose and other textile fila-  
ments and fibres such as cotton, wool, silk, flax,  
regenerated cellulose made by the cupram-  
monium or viscose methods, and other similar  
fibres or filaments. When applying this inven-  
tion to warps or fabrics, it is only necessary that 30  
the same contain some yarns consisting of or-  
ganic esters of cellulose or some yarns containing  
filaments or fibres of organic esters of cellulose.  
Thus, warps and fabrics may be made by alter-  
nating or putting in any sequence yarns contain-  
ing organic esters of cellulose and yarns made 35  
of other textile materials.

The yarns, warps or fabrics may be caused to  
be sensitized by contacting the same continuously 40  
or periodically with a furnishing device supplying  
a saponifying agent to the yarn in sufficient  
amount and concentration to etch the surface of  
the filaments by the saponifying agent. These  
sensitized yarns may be caused to develop a high 45  
degree of saponification in the parts sensitized by  
a treatment with a soap solution or other solu-  
tion having a pH value between 8 and 10.5. The  
amount of saponification necessary to sensitize  
the filaments to saponification in baths may be 50  
very light and to an extent that they lose only  
from two to 7% of their weight. This very light  
saponification, although capable of being de-  
veloped in later treatments to a very heavy sa-  
ponification, is, nevertheless, so light that it is 55

difficult to observe at the stage of the application of the saponifying agent to the yarn. In accordance with my invention, however, there is incorporated with the saponifying agent a colored organic material that has no effect on the organic esters of cellulose or upon the saponified organic esters of cellulose and that is readily washable from the yarns, warps or fabrics. By this means the operator may readily see how much of the area is being contacted by the saponifying agent and by comparison of color ascertain the differential degrees of saponification on those parts contacted.

The sensitizing or saponifying agent employed to treat the yarns, filaments or fabrics containing the organic ester of cellulose may be any suitable saponifying agent having a pH value of from 10.5 to 14. Any suitable basic solution may be employed for this purpose, such as an aqueous solution or an alcoholic solution of an alkali hydroxide, for instance, sodium hydroxide or potassium hydroxide, an aqueous solution of ammonium hydroxide, a salt of a strong base, such as ammonia or alkali, and a weak acid such as organic acids, organic compounds having a basic reaction, etc. Examples of salts of a strong base and organic acids which may be employed for this invention are sodium acetate, potassium acetate, etc. Examples of organic bases that may be employed as the sensitizing or saponifying agent are the primary, secondary and tertiary amines, for instance, ethanol amine, methanol amine, di-methanol amine, di-ethanol amine, tri-methanol amine and tri-ethanol amine. Also, quaternary ammonium bases may be employed, for instance, tetra methyl ammonium hydroxide, tetra ethyl ammonium hydroxide, etc. These may be applied to the yarn from aqueous solutions, which solutions may be of any suitable concentration such that the pH value of the solution is above 10.5.

With any of the above listed or similar saponifying agents there may be mixed an organic substance having a distinct color. This organic substance is to be of a type that is not reduced to a colorless liquid in strongly basic solutions when mixed with the same and held in contact with the same for long periods of time, for instance, one day to three weeks. In this respect the material is to be considered inert if it does not lose its color or appreciably change color over a period of three weeks. Furthermore, the colored organic material should be selected such that it has no dyeing effect upon the textile materials to which it is applied and should preferably be merely a fugitive tint capable of being removed easily, by scouring, from the material. Another property desirable in the organic coloring material is that it be easily removed by cold scouring treatments that may or may not contain soap. Examples of suitable colored organic materials for the treatment of textile materials containing organic esters of cellulose that are to be saponified are Xylene Light Yellow 2G (Color Index No. 639), Tartrazine (Color Index No. 640), Amidonaphthol Red G (Color Index No. 31) and Fast Acid Magenta B (Color Index No. 30). The colored organic material may have the chemical formula of sodium salt of 4-p-sulpho-benzene-azo-1-o-m-di-chloro-p-sulpho-phenyl-3-methyl-5-hydroxy-pyrazol, the sodium salt of benzene-azo-8-acetyl-amino-1-naphthol-3:6-di-sulphonic acid, the sodium salt of benzene-azo-8-amino-1-naphthol-3:6-di-sulphonic acid or organic materials of similar formula.

The modifying agent to be applied to the yarn

may be any suitable furnishing device such as a wick, roller or disc for individual yarns or a printing machine for warps and fabrics. The treating composition may contain any suitable concentration of the basic saponifying material and the colored organic material. When employing alkali hydroxides as the basic substance, the modifying agent or treating composition may contain from 10 to 30% by weight of same and to this may be added from 5 to 5 parts by weight of the colored organic material. The mixture of saponifying agent, colored organic material and carrier which may be either water, alcohol or similar substance, may be applied to the textile materials in amounts from  $\frac{1}{2}$  per cent to 8 per cent on the weight of the textile material.

For the purpose of further describing this invention and not as a limitation, the following example is given.

#### Example

Yarn formed of filaments of cellulose acetate travelling from a supply package to a take-up package at, for instance, about 100 metres per minute is caused to periodically contact with a furnishing roller. The furnishing roller may be caused to dip into the mixture consisting of 80 parts by weight of water, 20 parts by weight of sodium hydroxide and  $\frac{1}{2}$  part by weight of Amidonaphthol Red G. The yarn, where treated, will have a distinctive orange red color while the parts not treated will be of the white or natural color. The yarns so formed may be made into a warp or used as a filling in the formation of a fabric. After the fabric is formed, the same may be treated in a heated aqueous bath containing 10 grams per litre of soap. All trace of color is removed from the fabric and those parts of the yarn that were sensitized by the above saponifying action are developed to an extent of saponification such that they have lost from 10 to 20% by weight and their affinity for dye materials correspondingly changed.

Although the invention has been described with particular reference to saponifying or sensitizing yarns containing organic esters of cellulose, it is also applicable to other treatments of textile materials. For instance, this invention may be employed in the process where, acids, alcohols, solvents, softening agents, etc., are applied to yarns of artificial materials to deluster, reluster, shrink or otherwise change the properties of same. It may also be employed in the application of resist materials in resist printing operations.

The above description is merely given by way of illustration and many modifications may be made therein without departing from the spirit of my invention.

Having described my invention, what I desire to secure by Letters Patent is:

1. Method of treating textile materials containing organic esters of cellulose, which comprises intermittently applying to said cellulose ester materials a composition adapted to saponify at least the surface of said materials, said composition containing a colored organic material having no affinity for the unsaponified portion and fugitive to the saponified portion so as to render visible the saponified portion by coloring the same.

2. Method of treating textile materials containing cellulose acetate, which comprises intermittently applying to said cellulose acetate materials a composition adapted to saponify at least the surface of said materials, said composition

containing a colored organic material having no affinity for the unsaponified portion and fugitive to the saponified portion so as to render visible the saponified portion by coloring the same.

5. Method of treating textile materials containing organic esters of cellulose, which comprises intermittently applying to said cellulose ester materials a composition containing an alkali hydroxide adapted to cause at least partial saponification of said materials, said composition also containing a colored organic material having no affinity for the unsaponified portion and fugitive to the saponified portion so as to render visible the saponified portion by coloring the same.

10. 6. Method of treating textile materials containing cellulose acetate, which comprises intermittently applying to said cellulose acetate materials a composition containing an alkali hydroxide adapted to cause at least partial saponification of said materials, said composition also containing a colored organic material having no affinity for the unsaponified portion and fugitive to the saponified portion so as to render visible the saponified portion by coloring the same.

15. 7. Method of treating textile materials containing cellulose acetate, which comprises intermittently applying to said cellulose acetate materials a composition containing an alkali hydroxide adapted to cause at least partial saponification of said materials, said composition also containing a colored organic material having no affinity for the unsaponified portion and fugitive to the saponified portion by coloring the same.

20. 8. Method of treating textile materials containing cellulose acetate, which comprises intermittently applying to said cellulose acetate materials a composition containing an alkali hydroxide adapted to cause at least partial saponification of said materials, said composition also containing a colored organic material having no affinity for the unsaponified portion and fugitive to the saponified portion by coloring the same.

25. 9. Method of treating textile materials containing cellulose acetate, which comprises intermittently applying to said cellulose acetate materials a composition containing an alkali hydroxide adapted to cause at least partial saponification of said materials, said composition also containing a colored organic material having no affinity for the unsaponified portion and fugitive to the saponified portion by coloring the same.

30. 10. Method of treating textile materials containing cellulose acetate, which comprises intermittently applying to said cellulose acetate materials a composition containing an alkali hydroxide adapted to cause at least partial saponification of said materials, said composition also containing a colored organic material having no affinity for the unsaponified portion and fugitive to the saponified portion by coloring the same.

fication of said materials, said composition also containing a dyestuff having no affinity for the unsaponified portion and fugitive to the saponified portion and substantially unaffected by strong solutions of alkali hydroxides and adapted to color said textile material to render visible the saponified portion.

5. 11. Method of treating textile materials containing organic esters of cellulose, which comprises intermittently applying to said cellulose ester materials a composition containing an alkali hydroxide adapted to cause at least partial saponification of said materials, said composition also containing an organic coloring matter, selected from the group consisting of Xylene Light Yellow 2G, Tartrazine, Amidonaphthol Red G and Fast Acid Magenta B, so as to render visible the saponified portion of the materials.

10. 12. Method of treating textile materials containing cellulose acetate, which comprises intermittently applying to said cellulose acetate materials a composition containing an alkali hydroxide adapted to cause at least partial saponification of said materials, said composition also containing an organic coloring matter, selected from the group consisting of Xylene Light Yellow 2G, Tartrazine, Amidonaphthol Red G and Fast Acid Magenta B, so as to render visible the saponified portion of the materials.

15. WILLIAM WHITEHEAD. 30

5

10

15

20

25